

Feb. 6, 1940.

G. H. SMITH ET AL

2,189,301

BLASTING INITIATOR

Filed Nov. 19, 1936



*Fig. 1*

*Fig. 2*

*Fig. 3*

*Gilbert H. Smith*  
*Carl B. Van Winter* INVENTORS  
BY *Benton C. Bull*  
ATTORNEY.

## UNITED STATES PATENT OFFICE

2,189,301

## BLASTING INITIATOR

Gilbert H. Smith, Woodbury, and Carl B. Van Winter, Wenonah, N. J., assignors to E. I. du Pont de Nemours & Company, Wilmington, Del., a corporation of Delaware

Application November 19, 1936, Serial No. 111,582

## 13 Claims.

(Cl. 52-2)

The present invention relates to electric blasting initiators and more particularly to a new and improved ignition composition for the same.

Electric blasting initiators may be conveniently classified into two general types, namely, caps and squibs, depending on the character of the main explosive charge with which they are employed. The electric blasting cap serves to detonate high explosives of the dynamite type, whereas the electric squib is employed to initiate deflagrating explosives, such as black powder, where a flame-producing means is required. Both types, however, employ ignition compositions. In the case of the blasting cap the ignition composition serves to initiate a detonating base charge, whereas in the squib it is employed as the flame-producing base charge which ignites the black powder.

Ignition compositions suitable for use in either electric detonators or electric squibs should possess low uniform firing properties which can be readily duplicated in manufacturing operations. For electric squibs the ignition composition should possess, in addition to the low firing current properties, the ability to develop a hot flame of considerable duration on combustion. This property is required since in wet coal mines it is often necessary to ignite moist pelleted powder. Although some ignition compositions possess one or the other of these necessary properties, it is well recognized in the art that few materials are available which have all the required characteristics to the desired degree.

The object of the present invention is a new and improved ignition composition. A further object is such an ignition composition which is satisfactory with respect to low firing current and which produces a hot flame of considerable duration. A further object is a new and improved electric squib capable of igniting moist pelleted black powder. Further objects will be apparent from the detailed description of our invention which follows.

We have found that the foregoing objects may be accomplished by employing an ignition composition comprising smokeless powder, or smokeless powder and an oxidizing agent, preferably in the form of a grained loose charge, the smokeless powder being desirably ground. We have discovered further that the ignition properties are very desirably improved by incorporating therewith certain finely divided reductive fuels. For the purpose of our invention a great number of reductive fuels may be used, for example readily oxidizable, atmospherically stable metals or

metalloids, such as selenium, tellurium, zirconium, magnesium, aluminum and the like. Alloys as well as elementary metals may be employed, for example calcium silicide. Other readily oxidizable, atmospherically stable reductive fuels may be used in place of the metals, for example, sulfur and the like.

In order to disclose the nature of our invention more clearly, reference is made to the accompanying Table I, which illustrates preferred examples of ignition compositions in accordance with our invention.

Table I

| Example | Composition         |                         | Metal or<br>metalloid  |
|---------|---------------------|-------------------------|------------------------|
|         | Smokeless<br>powder | Oxidizing<br>agent      |                        |
| I       | Percent<br>100      | Percent<br>0            | Percent<br>0           |
| II      | 80                  | 20 (KClO <sub>4</sub> ) | 0                      |
| III     | 50                  | 42 (BaO <sub>2</sub> )  | 8 (CaSi <sub>2</sub> ) |
| IV      | 50                  | 47 (BaO <sub>2</sub> )  | 3 (S)                  |
| V       | 50                  | 49 (BaO <sub>2</sub> )  | 10 (Se)                |
| VI      | 50                  | 39 (BaO <sub>2</sub> )  | 11 (Zr)                |

In addition to the oxidizing agents indicated in the foregoing table, we may employ lead dioxide, potassium nitrate, barium nitrate and many other oxidizing agents.

In order further to illustrate the nature of our invention, reference is made to the accompanying drawing which represents preferred embodiments thereof. It is understood, however, that this is done solely by way of illustration and is not to be regarded as a limitation upon the scope of our invention.

Referring generally to the drawing, Figure 1 is a vertical elevation of an electric blasting cap, while Figures 2 and 3 are similar views of closed shell electric squibs. Corresponding parts of the different figures are represented by similar characters referred to in the following description.

In the drawing the numeral 1 represents a metal shell of any suitable material, such as aluminum, copper or the like. In Figure 1, a base charge 2 of detonating material is placed in the bottom of the shell and a primary charge 3, capable of initiating said base charge, is superposed thereon. Above the primary charge 3 is the loose ignition composition 4 in accordance with the present invention, for example the composition III of Table I. The bridge wire 5, between the leading wires 6, is embedded in the ignition composition 4. The leading wires 6 are

held in position by the bridge plug 7 and the shell is closed by the waterproofing composition 3 and the usual sulfur seal 9.

Figure 2 illustrates an electric squib in accordance with our invention. The shell 1 contains the base charge 2 of suitable deflagrating material, such as black powder. The base charge 2 is covered by a loose ignition charge 4 in accordance with our invention, for example the composition IV of Table I.

Figure 3 illustrates an electric squib differing slightly in construction from that shown in Figure 2, in that a single base charge 4 is employed. This base charge 4 may consist of any of the compositions in accordance with our invention, for example the composition V of Table I.

The firing currents necessary to ignite squibs having the foregoing ignition compositions range from 0.330 to 0.365 ampere, and due to the fact that the ignition compositions produce a hot flame of considerable duration the electric squibs in accordance with our invention are capable of igniting moist black powder pellets. The compositions disclosed can be consistently reproduced in large scale manufacture to give initiators having a high degree of uniformity in ignition properties.

Although we prefer to employ the compositions of our invention as ignition charges in electric squibs, either alone or as a primary charge, they may be used in electric blasting initiators generally as ignition charges, as illustrated in Figure 1 or the drawing. Although we may employ our ignition compositions generally in electric blasting initiators, we find them particularly advantageous when used in closed shell electric squibs provided with a bridge wire of slow fusing properties, as described and claimed in the copending application of Lawton A. Burrows and Carl B. Van Winter, Serial No. 111,581 filed November 19, 1936.

In the foregoing detailed description of our invention, it is apparent that many variations can be made without departing from the spirit and scope thereof. We intend, therefore, to be limited

only in accordance with the following patent claims.

We claim:

1. An electric blasting initiator containing an ignition composition comprising smokeless powder, an oxidizing agent, and at least one member of the group of reductive fuels consisting of sulfur, calcium silicide and readily oxidizable, atmospherically stable metals and metalloids. 5
2. A closed shell electric squib containing a loose ignition composition comprising smokeless powder, an oxidizing agent, and at least one member of the group of reductive fuels consisting of sulfur, calcium silicide and readily oxidizable, atmospherically stable metals and metalloids. 10
3. A closed shell electric squib containing a loose ignition composition comprising smokeless powder, an oxidizing agent, and calcium silicide. 20
4. A closed shell electric squib containing a loose ignition composition comprising smokeless powder, an oxidizing agent, and sulfur. 25
5. The electric squib of claim 2, wherein the reductive fuel is selenium.
6. The electric squib of claim 2, wherein the reductive fuel is zirconium. 30
7. The electric squib of claim 2, wherein the oxidizing agent is barium peroxide.
8. An electric blasting initiator containing an ignition composition consisting of smokeless powder and an oxidizing agent. 35
9. A closed shell electric squib containing a loose ignition composition consisting of smokeless powder and an oxidizing agent.
10. The electric squib according to claim 9, wherein the oxidizing agent is barium peroxide. 40
11. The electric squib according to claim 9, wherein the oxidizing agent is potassium chlorate.
12. The electric squib according to claim 9, wherein the oxidizing agent is potassium nitrate.
13. An electric blasting initiator containing an ignition composition consisting of ground smokeless powder.

GILBERT H. SMITH.

CARL B. VAN WINTER.

45